# EUROPEAN PATENT SPECIFICATION

(11) **EP 2 896 054 B1**
(45) Date of publication and mention of the grant of the patent: **24.04.2019**
(21) Application number: 13771661.9
(22) Date of filing: 11.09.2013
(51) Int. Cl.: H01B 7/295, H01B 19/04, H01B 11/06

(54) **FOAMED SEPARATOR SPLINES FOR DATA COMMUNICATION CABLES**
GESCHÄUMTE TRENNKEILE FÜR DATENKOMMUNIKATIONSKABEL
LANGUETTES SÉPARATRICES EXPANSÉES POUR CÂBLES DE COMMUNICATIONS DE DONNÉES

(30) Priority: 11.09.2012 US 201261699532 P; 15.03.2013 US 201313843208
(43) Date of publication of application: 22.07.2015
(73) Proprietor: SABIC Global Technologies B.V., 4612 PX Bergen op Zoom (NL)
(72) Inventor: TRYSON, Glen Robert, Pittsfield, Massachusetts 01201 (US); RICE, Brian, Huntersville, North Carolina 28078-6468 (US)
(74) Representative: Office Freylinger
(86) International application number: PCT/US2013/059203
(87) International publication number: WO 2014/043194

(56) References cited:
- WO-A1-01/41158
- WO-A2-2008/079263
- US-A1- 2005 199 415
- US-A1- 2009 163 609
- US-A1- 2010 200 269

## Description

### Background of the Invention

Disclosed herein are foamed, electrically insulating separator splines for communication cables, communication cables incorporating the same, the processes for production thereof and use of such cables.

Current communication cables are formed of "twisted pairs" of conductors, usually metallic conductors, such as copper wire. These electrical conductors may each be covered with a nonconductive covering, such as synthetic polymers, natural or synthetic rubbers, and blends of electrically non-conductive materials. The resultant individual electrical conductors are then formed into the twisted pair, where at least two conductors are twisted forming interleaved spirals of conductors. When used to form communication cables, typically four twisted pairs are arranged about an electrically insulative isolator. Such an isolator is hereinafter referred to generically as a "separator spline." In particular, a "separator spline" is an isolator having a four-arm shape, such as a cross (₊-shape), or X-shape, or a, and a flat tape-shape with each twisted pair lying in the space between the arms. However, the separator spline may also take other forms, as discussed further below. The purpose of the separator spline is to reduce "cross-talk" between each of the twisted pairs of electrical conductors, especially at high data transmission rates. The assembled separator spline and sets of twisted pairs can be covered in a sheath to form the completed communication cable.

US 2010/200269 A1 describes a separator for a communication cable that comprises a body that includes at least first and second segments adapted to define a plurality of quadrants in the communication cable. The segments are substantially perpendicular to each other and define a junction point of the segments. Each of the segments includes a main portion and a terminal end remote from the junction point of the segments. Each of the terminal ends has a shape such that each of the terminal ends is wider than the main portions of the segments. At least one air pocket is defined between the terminal ends of the segments. The air pocket includes a gap sized such that the air pocket is substantially enclosed.

WO 2008/079263 describes a process for making an extruded foamable composition where the foamable composition includes a partially-crystalline melt processible perfluoropolymer and a foam nucleating package. The process makes a foamed product having uniform foam cell size at high speeds without loss of product quality.

The current materials of choice for the electrically insulative isolators are fluoropolymers or polyolefins, depending on cable construction and performance requirements.

In the present environment, the use of any type of halogenated compounds, especially fluorinated compounds presents an environmental hazard to be avoided. On the other hand, materials such as polyolefins present fire and smoke hazards, especially when used in an electrical environment. Thus, there is a need for separator splines which do not possess the detriments of the known separator spline materials.

### Summary of the Invention

The invention provides an extruded separator spline of indeterminate length for separating at least two pairs of twisted conductors comprising an extrudate having an indeterminate length; said extrudate having a central longitudinal axis along its indeterminate length; and wherein the extrudate is formed of a foamed, polymeric, halogen-free material and further wherein the extrudate has
a. a shape having four arms emanating from the central longitudinal axis; the extrudate further comprising a cross-section without a continuous void along either the longitudinal axis or in any of said four arms; each of the arms being of uniform dimension from the longitudinal axis towards a terminal end of each arm; each of the arms being arranged in an angular disposition relative to the other arms of the extrudate and adjacent arms defining a space therebetween such that a twisted pair of conductors can nest in the space without extending beyond the terminal ends of the adjacent arms; or
b. a shape being selected from the group consisting of a rod, a star, and a bar; a periphery of each of the rod, the star and the bar having a plurality of cavities extending from the periphery into the body of the rod, the star and the bar; said cavities being of a size and shape to house within the cavity a twisted pair of conductors; the extrudate further comprising a cross-section without a continuous void along the longitudinal axis, and wherein the extrudate forms a separator spline suitable to isolate at least two twisted pair of conductors in a different cavity of said plurality of cavities.

The invention provides a separator spline which is a non-halogen containing polymer having excellent smoke, flame and toxicity properties.

In an embodiment, the separator spline is formed of a polymeric material having excellent smoke flame and toxicity properties, such as polyetherimide (PEI), a polyetherimide/polysiloxane copolymer, a thermoplastic-elastomer-modified-polyphenylene-ether blend and combinations thereof.

In a further embodiment, the separator spline is formed of a reduced density material, such as foamed polyetherimide (PEI), a foamed polyetherimide/polysiloxane copolymer, a foamed thermoplastic-elastomer-modified-polyphenylene-ether blend, and combinations thereof.

In a further embodiment foamed separator spline can be manufactured in indefinite lengths of up to 5000 meters and longer by continuous extrusion of a composition comprising polyetherimide (PEI), a polyetherimide/polysiloxane copolymer, a thermoplastic-elastomer-modified-polyphenylene-ether blend and combinations thereof, with a blowing agent, and optionally, a nucleating agent.

In a further embodiment an indefinite length, foamed separator spline can be manufactured by feeding preformed pellets of polyetherimide (PEI), a polyetherimide/polysiloxane copolymer, a thermoplastic-elastomer-modified-polyphenylene-ether blend and combinations thereof, with a blowing agent, and optionally, a nucleating agent, into a single screw extruder with a cross (₊-shape) or "X"-shaped die to produce foamed extrudate, which can be drawn down, in a profile extrusion process.

In still further embodiments, the foamed separator spline can be combined with two or more twisted pairs, preferably four twisted pairs, of conductors nested in the spaces between the arms of the foamed separator spline , and the foamed isolator and twisted pairs being enclosed in a sheath to provide a lightweight non-halogen containing, data communication cable of low smoke, flame and toxicity properties, excellent in dielectric constant to reduce cross-talk between twisted pairs, suitable for use in high speed data transmission, and of acceptable compressive strength for use as data communication cables and components of data systems.

### Brief Description of the Drawings

Fig. 1 is a pictorial representation of a prior art data communication cable;
Fig. 2 is a schematic representation of an "X" or cross(+)-shaped separator spline according to the invention;
Fig. 3 is a cross-sectional, schematic representation of an alternative shape for the separator spline of the present invention in the form of a rod;
Fig. 4 is a cross-sectional, schematic representation of a further alternative shape for the separator spline according to the present invention in the form of a star;
Fig. 5 is a cross-sectional, schematic representation of a further alternative shape for the separator spline according to the present invention in the form of a tube; and
Fig. 6 is a cross-sectional, schematic representation of a further alternative shape for the separator spline according to the present invention in the form of a flat rectangular shape.

### Detailed Description of the Preferred Embodiments

As shown in Fig. 1, a prior art data communication cable 10 is formed of a fluoropolymer separator spline 12 into which four twisted pairs 13, 14, 15 and 16 of conductors are nested. A sheath 18 surrounds the separator spline 12 and twisted pairs 13, 14, 15 and 16 to complete the communication cable 10. Each conductor 20 of the twisted pair may be independently covered in an electrically insulated manner. As an alternative to the fluoropolymer, a polyolefin can be used as the material for separator spline 12.

However, halogenated compounds (F, Cl, Br), may be environmentally harmful. Polyolefins present smoke, flame and toxicity hazards, especially in the electrical environment.

Thus, the present inventors have discovered that PEI can replace halogenated materials for improved smoke, flame and toxicity (SFT) properties meeting, or exceeding, regulatory requirements for data communications cable, e.g., the Underwriter's Laboratory Standard UL-910 Plenum Test, or NFPA 262. Although PEI is an electrically insulating material, it was further discovered that the dielectric constant of the PEI could be improve by introducing a chemical or physical blowing agent into the PEI to reduce its density and improve its dielectric constant. Density reduction of as little as 3% demonstrated improvement in dielectric constant. Density can be reduced even further until the physical properties of the resultant foamed separator spline (which can also be referred to as an "isolator") are compromised, such as loss of mechanical integrity or buckling when bent.

When the term "halogen-free" is used to describe a polymer, the term means that the polymer does not contain halogen atoms in the polymeric chain and no compounds added to the formulation which contain non-trace levels of halogen.

The present inventors have discovered that density reduction of from about 3% to about 62% represents the operative range with density reduction of from about 3% to about 55% being preferred. It is to be understood that dielectric performance of the separator spline improves as density decreases. The dielectric constant of solid (unfoamed) PEI is about 3.15 and the density reductions according to the invention can yield dielectric constants on the order of about 2.0.

Foaming of the PEI, or other polymers/copolymers or blends, suitable for use in the invention, can be achieved during melt processing into a shape suitable for the separator spline.

The separator spline 30 according to the invention is formed of a PEI (exemplified by ULTEM 1000, commercially available from SABIC Innovative Plastics of Pittsfield, Massachusetts) which, during melt processing, is foamed by the addition of a chemical or physical blowing agent. A suitable blowing agent is dihydrooxadazinone in a PEI carrier, commercially available as ULTEM FUL-C20, from SABIC Innovative Plastics of Pittsfield, Massachusetts. Preferably, a nucleating agent, such as talc, (commercially available as Ultra Talc 609 from Specialty Minerals Inc. of Bethlehem, PA), is included for improved bubble formation. In a most preferred embodiment, the PEI and nucleating agent have been previously processed in a compounding extruder to form pellets, which pellets are the feedstock for the extrusion process forming the separator spline extrudate. The nucleating agent can optionally be present, and when present, is preferably present in an amount of about 0.5% by weight, based on the weight of the PEI. In another embodiment, the amount of the nucleating agent can range from about 0.1 to 10% by weight, based on the weight of the PEI When used, the blowing agent is preferably present in an amount of about 0.25% to about 1.0% by weight. In another embodiment, the amount of the blowing agent can range from about 0;05% to about 1.0%, by weight.

The present inventors have found that the resultant separator spline can be made from a PEI providing desirable smoke, flame and toxicity performance without halogen-containing materials. Furthermore, because the PEI is foamed during the forming of the separator spline , the presence of bubbles, which have a lower dielectric constant than that the neat resin, improves the dielectric constant of the separator spline over neat PEI to further inhibit cross talk between the twisted pairs, as well as reducing overall part weight without compromising physical properties of the resultant cable and providing a higher compressive strength as compared to fluoropolymers and polyolefins, improving the functionality of the separator spline to hold the conductors apart.

The separator spline in a preferred form comprises a separator spline having a length ranging from 1 meter to 5000 meters and a cross sectional dimension ranging from 0.1 mm to 5 mm, and a thickness ranging from 0.1 to 5 mm.

The foamed separator spline exhibits a compressive strength ranging from 15 to less than 124 MPa, preferably a compressive strength of 27 to 84 MPa.

Although we have exemplified twisted pairs of conductors, it is to be expressly understood that the number of twisted pairs of conductors which are separated by the separator spline of the present invention is non-limiting and may typically range from two to sixteen twisted pairs.

Fig. 3 illustrates separator spline 32 in the form of a rod having numerous cavities 34, 35, 36 to act as receptacles for a twisted pair. Fig. 4 shows the shape of the separator spline 42 as a star with several spaces 44, 45, 46 between the points 47, 48, 49 to accept a twisted pair. Fig 5 illustrates a tube 52 having numerous cavities 54, 55, 56 to accept a twisted pair of conductors. Fig. 6 illustrates a flat rectangular shape 62 having numerous cavities 64, 65, 66 to accept a twisted pair of conductors. In another embodiment, flat separator splines according to our invention has no cavities.

Technologies to foam PEIs are described in published application US2007/0149629 A1, EP 0373402, U.S. Patents 4,543,368; 4,683,247; 4,980,389; 5,064,867; 5,135, 959; 5,234,966 and 6,057, 379, the entire disclosures of which are herein incorporated by reference. Preferred polyimides include polyetherimides and polyetherimide copolymers. The polyetherimide can be selected from (i) polyetherimide homopolymers, e.g., polyetherimides, (ii) polyetherimide co-polymers, e.g., polyetherimide siloxane, and (iii) combinations thereof. Polyetherimides are known polymers and are sold by SABIC Innovative Plastics under the ULTEM®* and SILTEM* brands (Trademark of SABIC Innovative Plastics IP B.V.).

In an embodiment, the polyetherimides are of formula (1): wherein a is more than 1, for example 10 to 1,000 or more, or more specifically 10 to 500.

The group V in formula (1) is a tetravalent linker containing an ether group (a "polyetherimide" as used herein) or a combination of an ether groups and siloxane groups (a "polyetherimide/siloxane"). Such linkers include but are not limited to: (a) substituted or unsubstituted, saturated, unsaturated or aromatic monocyclic and polycyclic groups having 5 to 50 carbon atoms, optionally substituted with ether groups, siloxane groups, or a combination of ether groups and siloxane groups; and (b) substituted or unsubstituted, linear or branched, saturated or unsaturated alkyl groups having 1 to 30 carbon atoms and optionally substituted with ether groups or a combination of ether groups, siloxane groups; or combinations comprising at least one of the foregoing. Suitable additional substitutions include, but are not limited to, ethers, amides, esters, and combinations comprising at least one of the foregoing.

The R group in formula (1) includes but is not limited to substituted or unsubstituted divalent organic groups such as: (a) aromatic hydrocarbon groups having 6 to 20 carbon atoms and derivatives thereof; (b) straight or branched chain alkylene groups having 2 to 20 carbon atoms; (c) cycloalkylene groups having 3 to 20 carbon atoms, or (d) divalent groups of formula (2): wherein Q¹ includes but is not limited to a divalent moiety such as -O-, -S-, -C(O)-, -SO₂-, - SO-, -C_{y}H_{2y}- (y being an integer from 1 to 5), and derivatives thereof.

In an embodiment, linkers V include but are not limited to tetravalent aromatic groups of formula (3): wherein W is a divalent moiety including -O-, -SO₂-, or a group of the formula -O-Z-O-wherein the divalent bonds of the -O- or the -O-Z-O- group are in the 3,3', 3,4', 4,3', or the 4,4' positions, and wherein Z includes, but is not limited, to divalent groups of formulas (4): wherein Q includes, but is not limited to a divalent moiety including -O-, -S-, -C(O),

-SO₂-, -SO-, -C_{y}H_{2y}- (y being an integer from 1 to 5), and derivatives thereof.

In a specific embodiment, the polyetherimide comprise more than 1, specifically 10 to 1,000, or more specifically, 10 to 500 structural units, of formula (5): wherein T is -O- or a group of the formula -O-Z-O- wherein the divalent bonds of the -O- or the -O-Z-O- group are in the 3,3', 3,4', 4,3', or the 4,4' positions; Z is a divalent group of formula (3) as defined above; and R is a divalent group of formula (2) as defined above.

The polyetherimides can be synthesized by the reaction of the bis(phthalimide) (8) with an alkali metal salt of a dihydroxy substituted aromatic hydrocarbon of the formula HO-V-OH wherein V is as described above, in the presence or absence of phase transfer catalyst. Suitable phase transfer catalysts are disclosed in U.S. Patent No. 5,229,482, incorporated herein by reference. Specifically, the dihydroxy substituted aromatic hydrocarbon a bisphenol such as bisphenol A, or a combination of an alkali metal salt of a bisphenol and an alkali metal salt of another dihydroxy substituted aromatic hydrocarbon can be used.

In an embodiment, the polyetherimide comprises structural units of formula (5) wherein each R is independently p-phenylene or m-phenylene or a mixture comprising at least one of the foregoing; and T is group of the formula -O-Z-O- wherein the divalent bonds of the -O-Z-O- group are in the 3,3' positions, and Z is 2,2-diphenylenepropane group (a bisphenol A group).

The silicon polyetherimide can be any silicon-containing polyetherimide, which when used in accordance with the invention, enables the composition to exhibit a useful combination of improved flame retardancy, low smoke, and high impact strength properties, such that the compositions can pass the ASTM E 162 Standard Test Method for Surface Flammability of Materials Using a Radiant Heat Energy Source. Siloxane polyimide copolymers are a specific silicon polyetherimide that may be used in the blends of this invention. Examples of such siloxane polyimides are described in U.S. Patents 5,028,681, 4,808,686, 4,690,997, 4,404,350, 4,051,163, 4,011,279, 3,847,867, 3,833,546 and 3,325,450, the entire disclosures of which are herein incorporated by reference. Siloxane polyimides can be prepared by standard methods to make polyimides wherein at least a portion, generally from 5 to 70 wt. %, and optionally from 10 to 50 wt. %, of the imide is derived from siloxane containing diamines, siloxane containing dianhydrides or chemical equivalents thereof. Such siloxane polyimides include SILTEM*s, which can be obtained from SABIC Innovative Plastics (*Trademark of SABIC Innovative Plastics).

The siloxane polyimide can be prepared by any of the methods known to those skilled in the art, including the reaction of an aromatic bis(ether anhydride) of the Formula 6, with an organic diamine of the Formula 7,

H₂N-R-NH₂ (7),

wherein T is a divalent moiety selected from -O-, -S-, -C(O)-, SO₂-, -SO, a direct linkage, a fused ring linkage, or a group of the formula -O-Z-O- wherein the divalent bonds of the -Tor the -O-Z-O- group are in the 3,3', 3,4', 4,3', or the 4,4' positions, and wherein Z includes, but is not limited, (a) aromatic hydrocarbon radicals having about 6 to about 36 carbon atoms and halogenated derivatives thereof including perfluoroalkylene groups; (b) straight or branched chain alkylene radicals having about 2 to about 24 carbon atoms (c) cycloalkylene radicals having about 3 to about 20 carbon atoms, or (d) divalent radicals of the general Formula 8: wherein Q includes but is not limited to a divalent moiety selected from -O-, -S-, -C(O)-, - SO₂-, -SO-, -C_{y}H_{2y}- (y being an integer from 1 to 8), and fluorinated derivatives thereof, including perfluoroalkylene groups, and wherein at least a portion of the reactants, either dianhydride, diamine, or mixtures thereof, contain a siloxane functionality. The moiety R in Formula 2 includes but is not limited to substituted or unsubstituted divalent organic radicals such as: (a) aromatic hydrocarbon radicals having about 6 to about 36 carbon atoms and halogenated derivatives thereof; (b) straight or branched chain alkylene radicals having about 2 to about 20 carbon atoms; (c) cycloalkylene radicals having about 3 to about 24 carbon atoms, or (d) divalent radicals of the general Formula 8.

Examples of suitable diamine compounds are ethylenediamine, propylenediamine, trimethylenediamine, decamethylenediamine, 1,12-dodecanediamine, 2,5-dimethylheptamethylenediamine, 2, 2-dimethylpropylenediamine, N-methyl-bis (3-aminopropyl) amine, 3-methoxyhexamethylenediamine, 1,2-bis(3-aminopropoxy) ethane, bis(3-aminopropyl) sulfide, 1,4-cyclohexanediamine, bis-(4-aminocyclohexyl) methane, m-phenylenediamine, p-phenylenediamine, 2,4-diaminotoluene, 2,6-diaminotoluene, m-xylylenediamine, p-xylylenediamine, 2-methyl-4,6-diethyl-1,3-phenylene-diamine, 5-methyl-4,6-diethyl-1,3-phenylene-diamine, benzidine, 3,3'-dimethylbenzidine, 3,3'-dimethoxybenzidine, 1,5-diaminonaphthalene, bis(4-aminophenyl) methane, bis(2-chloro-4-amino-3, 5-diethylphenyl) methane, bis(4-aminophenyl) propane, 2,4-bis(p-amino-t-butyl) toluene, bis(p-amino-t-butylphenyl) ether, bis(p-methyl-o-aminophenyl) benzene, bis(p-methyl-o-aminopentyl) benzene, 1, 3-diamino-4-isopropylbenzene, bis(4-aminophenyl) sulfide, bis (4-aminophenyl) sulfone, bis(4-aminophenyl) ether and 1,3-bis(3-aminopropyl) benzene. Mixtures comprising at least one of the foregoing compounds may also be used. In some embodiments, diamino compounds are aromatic diamines, especially m- and p-phenylenediamine, sulfonyl dianilines, bis aminophenoxy benzenes, bis amino phenoxy sulfones and mixtures comprising at least one of the foregoing diamines.

Examples of specific aromatic bis anhydrides and organic diamines are disclosed in US Patents 3,972,902 and 4,455,410. Illustrative examples of aromatic bis anhydrides include: 3,3-bis[4-(3,4-dicarboxyphenoxy)phenyl]propane dianhydride; 4,4'-bis(3,4-dicarboxyphenoxy)diphenyl ether dianhydride; 4,4'-bis(3,4-dicarboxyphenoxy)diphenyl sulfide dianhydride; 4,4'-bis(3,4-dicarboxyphenoxy)benzophenone dianhydride; 4,4'-bis(3,4-dicarboxyphenoxy)diphenyl sulfone dianhydride; 2,2-bis[4-(2,3-dicarboxyphenoxy)phenyl]propane dianhydride; 4,4'-bis(2,3-dicarboxyphenoxy)diphenyl ether dianhydride; 4,4'-bis(2,3-dicarboxyphenoxy)diphenyl sulfide dianhydride; 4,4'-bis(2,3-dicarboxyphenoxy)benzophenone dianhydride; 4,4'-bis(2,3-dicarboxyphenoxy)diphenyl sulfone dianhydride; 4-(2,3-dicarboxyphenoxy)-4'-(3,4-dicarboxyphenoxy)diphenyl-2,2-propane dianhydride; 4-(2,3-dicarboxyphenoxy)-4'-(3,4-dicarboxyphenoxy)diphenyl ether dianhydride; 4-(2,3-dicarboxyphenoxy)-4'-(3,4-dicarboxyphenoxy)diphenyl sulfide dianhydride; 4-(2,3-dicarboxyphenoxy)-4'-(3,4-dicarboxyphenoxy)benzophenone dianhydride and 4-(2,3-dicarboxyphenoxy)-4'-(3,4-dicarboxyphenoxy)diphenyl sulfone dianhydride, pyromellitic dianhydride, biphenyl dianhydride, oxy diphthalic anhydride, sulfone diphthalic anhydride, hydroquinone diphthalic anhydride, resorcinol diphthalic anhydride and mixtures comprising at least one of the foregoing compounds.

In an embodiment, the polyetherimides include a polyetherimide thermoplastic composition, comprising: (a) a polyetherimide, and (b) a phosphorus-containing stabilizer, in an amount that is effective to increase the melt stability of the polyetherimide, wherein the phosphorus-containing stabilizer exhibits a low volatility such that, as measured by thermogravimetric analysis of an initial amount of a sample of the phosphorus-containing stabilizer, greater than or equal to 10 percent by weight of the initial amount of the sample remains unevaporated upon heating of the sample from room temperature to 300° C. at a heating rate of a 20° C. per minute under an inert atmosphere. In an embodiment, the phosphorous-containing stabilizer has a formula P-R'ₐ, where R' is independently H, alkyl, alkoxy, aryl, aryloxy, or oxy substituent and a is 3 or 4. Examples of such suitable stabilized polyetherimides can be found in U.S. Pat. No. 6,001,957, incorporated herein in its entirety.

As such, the invention includes an embodiment in which the separator spline comprises an amorphous polymer composition comprising (a) a polyetherimide, and (b) a phosphorus-containing stabilizer, in an amount that is effective to increase the melt stability of the polyetherimide, wherein the phosphorus-containing stabilizer exhibits a low volatility such that, as measured by thermogravimetric analysis of an initial amount of a sample of the phosphorus-containing stabilizer, greater than or equal to 10 percent by weight of the initial amount of the sample remains unevaporated upon heating of the sample from room temperature to 300° C. at a heating rate of a 20° C. per minute under an inert atmosphere. In an embodiment, the article is made such that the phosphorous-containing stabilizer has a formula P-Rₐ, where R' is independently H, alkyl, alkoxy, aryl, aryloxy, or oxy substituent and a is 3 or 4.

The polyimide siloxanes can also be prepared in a manner similar to that used for polyimides, except that a portion, or all, of the organic diamine reactant is replaced by an amine-terminated organosiloxane, for example of the Formula 9 wherein g is an integer from 1 to about 100, optionally from about 5 to about 50, and R' is an aryl, alkyl or aryl alky group of from 2 to 20 carbon atoms.

Some polyimide siloxanes may be formed by reaction of an organic diamine, or mixture of diamines, and the amine-terminated organosiloxane of Formula 9, and one or more dianhydrides. The diamino components may be physically mixed prior to reaction with the bis-anhydride(s), thus forming a substantially random copolymer. Alternatively block or alternating copolymers may be formed by selective reaction of 4 with dianhydrides to make polyimide blocks that are subsequently reacted together. In another instance the siloxane used to prepare the polyimide copolymer may have anhydride rather than amine functional end groups, for example as described in US Patent 4,404,350, the entire disclosure of which is herein incorporated by reference.

In another embodiment the siloxane polyimide copolymer can be of Formula 10 wherein T, R' and g are described as above, n is from 5 to about 100 and Ar is an aryl or alkyl aryl group of from 6 to 36 carbons.

In some siloxane polyetherimides the diamine component of the siloxane polyetherimide copolymers may contain from about 5 to 70 wt.% of the amine-terminated organosiloxane of Formula 9 and from about 30 to 95 wt.% of the organic diamine of Formula 7. In some siloxane copolymers, the siloxane component contains from about 25 to about 40 wt. % of the amine or anhydride terminated organosiloxane.

In some embodiments the siloxane polyimides can be siloxane polyetherimides which contain aryl ether linkages that can be derived by polymerization of dianhydrides and/or diamines wherein at least a portion of the dianhydride or the diamine contains an aryl ether linkage. In some instances both the diamine and dianhydride will contain an aryl ether linkage and at least a portion of the diamine or dianhydride will contain siloxane functionality, for example as described above. In other embodiments the aryl ether linkage can be derived from dianhydrides such as bisphenol A diphthalic anhydride, biphenol diphthalic anhydride, oxy diphthalic anhydride or mixtures thereof. In still other siloxane polyetherimides the aryl ether linkages can be derived from at least one diamine containing aryl ether linkages, for example, diamino diphenyl ethers, bis amino phenoxy benzenes, bis amino phenoxy phenyl sulfones or mixtures thereof. Either the diamine or dianhydride may have aryl ether linkages or in some instances both monomers may contain aryl ether linkages.

The silicone polyetherimide can have from about 5 to about 50, from about 10 to about 40, or from about 20 to about 30 percent by weight dimethyl siloxane units.

The silicone polyetherimide can have less than about 100, less than about 75, or from 10 to about 50 ppm amine end groups;

The silicone polyetherimide can have a weight average molecular weight from about 5,000 to about 70,000, from about 10,000 to about 60,000, or from about 20,000 to about 50,000 Daltons.

The articles can be made by any suitable method. For instance, the separator splines can be made by extruding. In other embodiments, the separator splines can be made by a method for making an article comprising extruding, injection molding, compressing molding, machining, and/or film pressing. In another embodiment separator splines can be made by additive manufacturing techniques.

In embodiments where additive manufacturing techniques are used to make separator splines, our separator spline can be made by any suitable process that uses additive manufacturing strategies. In an embodiment, our invention includes a method for building a three-dimensional separator spline in an extrusion-based digital manufacturing system, the method comprising: providing a consumable filament of the polymeric material to the extrusion-based digital manufacturing system, the consumable filament having a length, an exterior surface, and a plurality of tracks along at least a portion of the length, wherein the plurality of tracks provide a fractal dimensionality for at least a portion of the exterior surface that is greater than two for a suitable length scale, e.g., a length scale between 0.01 millimeters and 1.0 millimeter; engaging teeth of a rotatable drive mechanism retained by the extrusion-based digital manufacturing system with the plurality of tracks of the consumable filament; feeding successive portions of the consumable filament with the rotatable drive mechanism to a liquefier retained by the extrusion-based digital manufacturing system, wherein successive teeth of the rotatable drive mechanism are continuously engaged with successive tracks of the plurality of tracks while feeding the successive portions of the consumable filament; melting the consumable filament in the liquefier to provide a melted consumable material; extruding the melted consumable material from the liquefier; and depositing the extruded consumable material in a layer-by-layer manner to form at least a portion of the separator spline, which can generate back pressure in the liquefier. The consumable filament can be made by any suitable geometry. In an embodiment, the consumable filament has a substantially cylindrical geometry with an average diameter ranging from about 1.143 millimeters to about 2.54 millimeters. In another embodiment, the consumable filament has a substantially rectangular cross-sectional profile. The plurality of tracks can be selected from rectangular tracks, parabolic tracks, worm-type tracks, corrugated tracks, textured tracks, impressed file-type tracks, herringbone-type tracks, sprocket tracks, edge-facing tracks, staggered tracks, and combinations thereof.

As such, our invention includes an embodiment in which the separator spline is made in an extrusion-based digital manufacturing system, the method comprising: providing a consumable filament of the polymeric material to the extrusion-based digital manufacturing system, the consumable filament having a length, an exterior surface, and a plurality of tracks along at least a portion of the length, wherein the plurality of tracks provide a fractal dimensionality for at least a portion of the exterior surface that is greater than two for a length scale between 0.01 millimeters and 1.0 millimeter; engaging teeth of a rotatable drive mechanism retained by the extrusion-based digital manufacturing system with the plurality of tracks of the consumable filament; feeding successive portions of the consumable filament with the rotatable drive mechanism to a liquefier retained by the extrusion-based digital manufacturing system, wherein successive teeth of the rotatable drive mechanism are continuously engaged with successive tracks of the plurality of tracks while feeding the successive portions of the consumable filament; melting the consumable filament in the liquefier to provide a melted consumable material; extruding the melted consumable material from the liquefier; and depositing the extruded consumable material in a layer-by-layer manner to form at least a portion of the separator spline. A suitable apparatus for carrying out this method is disclosed in U.S. Patent 8,236,227, the entire disclosure of which is herein incorporated by reference.

### Examples

The following Examples and Comparative Examples are not limiting but are provided to assist the ordinary worker skilled in the art to which this invention pertains to practice the best mode.

### Examples 1-5

The purpose of these Examples is to produce an extruded shape from foamed polyetherimide (PEI) which could be used as a separator spline in a cable construction.

Materials are as in Table A.

**Table A**

| COMPONENT | CHEMICAL DESCRIPTION | SOURCE, VENDOR |
|---|---|---|
| ULTEM 1000 | Polyetherimide (PEI) | SABIC |
| Talc | Ultra Talc 609 | SABIC |
| ULTEM FUL-C20 | A dihydrooxadiazinone in a PEI carrier - a chemical blowing agent | SABIC |

### Techniques and Procedures

ULTEM 1000 was combined with 0.5% talc by weight using a twin screw extruder and standard polyetherimide compounding conditions to produce a compound used in subsequent extrusion trials to produce foamed parts.

In the following Comparative and Examples 1-5 of the invention, an Akron single-screw extruder (2 inch screw diameter, L/D=24, 3:1 compression ratio) was used with an "X"-shaped die to produce neat (non-foamed) and foamed parts with a PEI polymer. Nominal dimensions of the die were 0.220 inch by 0.220 inch (designed to be used with polyethylene to produce a part 0.130 inch by 0.130 inch with a wall thickness of 0.018 inch when drawn down in a profile extrusion process). The extruder was operated with a temperature profile of 327-343-343-343°C, progressing from the feed zone to the die, at a screw speed of 25 rpm. Puller speed was varied to achieve target dimensions.

A blowing agent (ULTEM FUL-C20) (with 0.5 wt% talc) in various amounts was used in preparing the foamed separator spline s according to the invention.

### Example 1 (Comparative Example)

A polyetherimide (PEI), commercially available as ULTEM 1000 from SABIC Innovative Plastics was used as a baseline, with no blowing agent or introduced air bubbles (a neat resin). The PEI was fed to the Akron single screw extruder under the conditions specified above to obtain an "+"-shaped extrudate having a relative linear density of 100%, an apparent specific gravity of 1.27 and a density reduction of 0%. The weight of a 1 meter length of extrudate was 4.6669 gram. Its properties are as set forth in Table 1.

### Example 2

The same PEI as used in example 1 was combined with a blowing agent (ULTEM FUL-C20 from SABIC Innovative Plastics) in an amount of 11.4 g/4540 g PEI, and extruded in the Akron single screw extruder under the conditions specified above. The resultant extrudate exhibited a relative linear density of 91%, an apparent specific gravity of 1.23 and a density reduction of 3%. It exhibited a slight foaming. Its properties are as set forth in Table 1.

### Example 3

The same PEI as used in example 1 was combined with a blowing agent (ULTEM FUL-C20 from SABIC Innovative Plastics) in an amount of 17.1 g/4540 g PEI, and extruded in the Akron single screw extruder under the conditions specified above. The resultant extrudate exhibited a relative linear density of 79%, an apparent specific gravity of 1.01 and a density reduction of 21%. It exhibited foaming with good mechanical properties. Its properties are as set forth in Table 1.

### Example 4

The same PEI as used in example 1 was combined with a blowing agent (ULTEM FUL-C20 from SABIC Innovative Plastics) in an amount of 22.8 g/4540 g PEI, and extruded in the Akron single screw extruder under the conditions specified above. The resultant extrudate exhibited a relative linear density of 46%, an apparent specific gravity of 0.57 and a density reduction of 55%. It exhibited significant foaming but the separator spline buckled when bent. Its properties are as set forth in Table 1.

### Example 5

The same PEI as used in example 1 was combined with a blowing agent (ULTEM FUL-C20 from SABIC Innovative Plastics) in an amount of 45.4 g/4540 g PEI, and extruded in the Akron single screw extruder under the conditions specified above. The resultant extrudate exhibited a relative linear density of 42%, an apparent specific gravity of 0.48 and a density reduction of 62%. It exhibited loss of mechanical integrity, could not get into dimension with line speed. Its properties are as set forth in Table 1.

**TABLE 1**

| Run No. | FUL-C20 Loading | FUL-C20 Loading | Line Speed | Weight of 1 meter piece | Dim 1 | Dim 2 | Wall Thickness | Relative Linear Density | Apparent Specific Gravity | Density Reduction | Comments |
|---|---|---|---|---|---|---|---|---|---|---|---|
| | (%) | (g/4540 g polymer) | (m/sec) | (g) | (mm) | (mm) | (mm) | | | (%) | |
| 1 | 0.00 | 0 | 0.81 | 4.6669 | 3.28 | 3.23 | 0.64 | 100% | 1.27 | 0 | No blowing agent - baseline |
| 2 | 0.25 | 11.4 | 0.81 | 4.2701 | 3.05 | 3.20 | 0.58 | 91% | 1.23 | 3 | Slight foaming |
| 3 | 0.38 | 17.1 | 0.85 | 3.6906 | 3.28 | 3.30 | 0.61 | 79% | 1.01 | 21 | Foaming, mechanicals good |
| 4 | 0.50 | 22.8 | 1.61 | 2.1339 | 3.35 | 3.43 | 0.66 | 46% | 0.57 | 56 | Significant foaming, isolator buckles when bent |
| 5 | 1.00 | 45.4 | >1.61 | 1.9694 | 3.68 | 3.66 | 0.56 | 42% | 0.48 | 62 | Loss of mechanical integrity, couldn't get into dimension with line speed |

Examples 1-5 demonstrate the ability to produce a reduced density part from PEI that could function as a separator spline in a cable construction. With blowing agent loadings of 0.38% and 0.5%, density reductions of 21% and 56% respectively were achieved. Parts were produced which met targeted dimensions for the +-shape cross-section. One skilled in the art of profile extrusion die design and processing would be able to optimize equipment and process conditions to produce other specified dimensions.

Although we have described the extrusion of separator splines having a +-shape or an X-shape, and a flat tape-shape to separate each of four twisted pairs of conductors, it is within the scope of the invention to provide other shapes of isolators (separator splines) to serve to isolate different numbers of twisted pairs in data communication cables. These can take the form of a rod, a star configuration, a tube, or a flat rectangular shape.

### Example 6

The purposed of this example is to examine different chemical blowing agents to determine suitability for use with polyetherimide in an extrusion process. Materials are shown in Table B.

**Table B.**

| COMPONENT | CHEMICAL DESCRIPTION | SOURCE, VENDOR |
|---|---|---|
| ULTEM 1010 | Polyetherimide (PEI) | SABIC |
| ULTEM FUL-C20 | A dihydrooxadiazinone in a PEI carrier | SABIC |
| Safoam NPC-20 | Proprietary endothermic chemical blowing agent | Reedy International Corporation |
| Safoam RPC-40 | Proprietary endothermic chemical blowing agent | Reedy International Corporation |

### Techniques and Procedures

A Killion single-screw extruder (25 mm screw diameter, L/D=24, barrier screw design) was used with a circular (rod) die to produce foamed parts. Nominal dimension of the die opening was 1.0 mm. The extruder was operated with a temperature profile and screw speed as shown in Table 2. The extruded strand of material was allowed to collect on the floor below the die.

Different chemical blowing agents (detailed in the Materials Table B) were blended with ULTEM 1010 polyetherimide at a level of 2.0% by weight and passed through the extruder to produce a strand of foamed material.

Dimensions of extruded parts were measured using a standard set of calipers with precision of 0.001". Weights of extruded parts were determined using a Mettler analytical balance with precision of 0.0001 g. Apparent specific gravity and density reduction were calculated from these measurements.

Table 2 shows results from several extrusion runs with different chemical blowing agents added to PEI and extruded.

The runs in Table 2 demonstrate the efficacy of different chemical blowing agents for producing polyetherimide foam in an extrusion process. The ULTEM FUL-C20 compound is very effective, NPC-20 compound produces foam but is less effective, and RPC-40 is not suited for producing PEI foam.

### Example 7

The purpose of this Example is to examine the effects of adding a nucleating agent (talc) to polyetherimide and a chemical blowing agent to produce foam in an extrusion process. The materials shown in Table C were used.

**Table C**

| COMPONENT | CHEMICAL DESCRIPTION | SOURCE, VENDOR |
|---|---|---|
| ULTEM 1000 | Polyetherimide (PEI) | SABIC |
| Talc | Ultra Talc 609 | SABIC |
| ULTEM FUL-C20 | A dihydrooxadiazinone in a PEI carrier | SABIC |
| Safoam NPC-20 | Proprietary endothermic chemical blowing agent | Reedy International Corporation |

### Techniques and Procedures

ULTEM 1000 was combined with 0.5% talc by weight using a twin screw extruder and standard polyetherimide compounding conditions to produce a compound used in subsequent extrusion trials to produce foamed parts.

A Killion single-screw extruder (25 mm screw diameter, L/D=24, barrier screw design) was used with a circular (rod) die to produce foamed parts. Nominal dimension of the die opening was 1.0 mm. The extruder was operated with a temperature profile and screw speed as shown Table 3. The extruded strand of material was allowed to collect on the floor below the die.

Different chemical blowing agents (detailed in the Materials Table C) were blended with a polyetherimide /0.5% talc compound at a level of 2.0% by weight and passed through the extruder to produce a strand of foamed material.

Dimensions of extruded parts were measured using a standard set of calipers with precision of 0.001 inches. Weights of extruded parts were determined using a Mettler analytical balance with precision of 0.0001 g. Apparent specific gravity and density reduction were calculated from these measurements.

Table 3 shows results from extrusion runs with different chemical blowing agents added to a PEI/talc compound and extruded.

The runs in Table 3 illustrate that adding talc at a low level to polyetherimide and a chemical blowing agent results in a uniform foam when extruded. In addition to stabilizing the extrusion process, the nucleating agent may also enhance the degree of foaming for a given level of blowing agent.

### Example 8.

The purpose of Example 8 is to produce foamed parts in an extrusion process using a polyetherimide/siloxane copolymer (SILTEM* brand) with a chemical blowing agent. The materials in Table D were used.

**Table D.**

| COMPONENT | CHEMICAL DESCRIPTION | SOURCE, VENDOR |
|---|---|---|
| ULTEM 1000 | Polyetherimide (PEI) | SABIC |
| ULTEM STM1700 | Polyetherimide/siloxane copolymer | SABIC |
| ULTEM FUL-C20 | A dihydrooxadiazinone in a PEI carrier | SABIC |

### Techniques and Procedures

A Killion single-screw extruder (25 mm screw diameter, L/D=24, barrier screw design) was used with a circular (rod) die to produce foamed parts. Nominal dimension of the die opening was 1.0 mm. The extruder was operated with a temperature profile and screw speed as shown in Table 4. The extruded strand of material was allowed to collect on the floor below the die.

ULTEM FUL-C20 chemical blowing agent was blended with a polyetherimide/siloxane copolymer at a level of 2.0% by weight and passed through the extruder to produce a strand of foamed material.

Dimensions of extruded parts were measured using a standard set of calipers with precision of 0.001". Weights of extruded parts were determined using a Mettler analytical balance with precision of 0.0001 g. Apparent specific gravity and density reduction were calculated from these measurements.

Table 4 shows results from extrusion runs with polyetherimide and with a polyetherimide/siloxane copolymer plus chemical blowing agent.

The examples in Table 4 illustrate that ULTEM FUL-C20 is effective as a blowing agent for a polyetherimide/siloxane copolymer in an extrusion process. Based on the findings illustrated by Example 8, it is expected that the addition of talc to this system will improve the quality of the foam.

**TABLE 2**

| Run No. | Material | Extruder Temperature Settings | Screw | BA Level | Talc Level | Density | Density Reduction | Comments |
|---|---|---|---|---|---|---|---|---|
| | | Feed Zone ==> Die (C) | RPM | (Wt. %) | (Wt. %) | (g/cm^3) | (%) | |
| 0 | ULTEM 1010 | 316-327-327-327-327-332 | 10 | 0 | 0 | 1.27 | 0 | Baseline - No foaming |
| 1 | ULTEM 1010 + 2% FUL-C20 | 316-327-327-327-327-332 | 10 | 2 | 0 | 0.42 | 67 | Amount of foaming varying - possible incomplete mixing |
| 2A | ULTEM 1010 + 2% NPC-20 | 316-327-327-327-327-332 | 10 | 2 | 0 | 1.11 | 13 | Coarse bubbles - less foaming than FUL-C20 |
| 2B | ULTEM 1010 + 2% NPC-20 | 316-327-327-327-327-332 | 15 | 2 | 0 | 1.08 | 15 | Higher throughput - similar foaming |
| 3A | ULTEM 1010 + 2% RPC-40 | 316-327-327-327-327-332 | 10 | 2 | 0 | 1.27 | 0 | Low pressure and throughput rate. Clumping of ULTEM to BA pellets |
| 3B | ULTEM 1010 + 2% RPC-40 | 316-327-327-327-327-332 | 20 | 2 | 0 | --- | --- | No sample retained - not foaming much |

**TABLE 3**

| Run No. | Material | Extruder Temperature Settings | Screw | BA Level | Talc Level | Density | Density Reduction | Comments |
|---|---|---|---|---|---|---|---|---|
| | | Feed Zone ==> Die (C) | RPM | (Wt. %) | (Wt. %) | (qm/cm^3) | (%) | |
| 1 | ULTEM 1000 | 316-332-343-343-343-343 | 8 | 0 | 0 | 1.27 | 0 | Baseline - No foaming |
| 2 | ULTEM 1000 + 2.0% FUL-C20 | 316-332-332-335-335-338 | 8 | 2 | 0 | --- | --- | Foaming variable - sample not consistent - had to lower temps |
| 3 | ULTEM 1000 + 0.5% talc + 2.0% FUL-C20 | 316-332-332-335-335-338 | 8 | 2 | 0.5 | 0.48 | 63 | Smaller, more uniform bubbles with talc |
| 4 | ULTEM 1000 + 0.5% talc + 2.0% NPC-20 | 316-332-332-335-335-338 | 8 | 2 | 0.5 | 0.69 | 46 | Smaller, more uniform bubbles with talc - less density reduction compared to FUL-C20 |

**Table 4**

| Run No. | Material | Extruder Temperature Settings | Screw | BA Level | Talc Level | Density | Density Reduction | Comments |
|---|---|---|---|---|---|---|---|---|
| | | Feed Zone ==> Die (C) | RPM | (Wt. %) | (Wt. %) | (gm/cm^3) | (%) | |
| 1 | ULTEM 1000 | 316-332-332-335-335-338 | 8 | 0 | 0 | 1.27 | 0 | Baseline - No foaming |
| 5 | ULTEM STM1700 | 299-299-304-304-304-304 | 10 | 0 | 0 | 1.20 | 0 | Baseline - No foaming |
| 6 | ULTEM STM1700 + 2.0% FUL-C20 | 299-299-304-304-304-304 | 10 | 2 | 0 | 0.55 | 54 | Coarse bubbles |
| 6A | ULTEM STM1700 + 2.0% FUL-C20 | 299-299-304-304-304-304 | 20 | 2 | 0 | 0.59 | 51 | Coarse bubbles |

### Example 9

The purpose of this example was to make a separator spline with additive manufacturing techniques.

### Techniques and Procedures

The separator spline was made in an extrusion-based digital manufacturing system as follows. A consumable filament of polyetherimide sold commercially as ULTEM 9085, manufactured and sold by SABIC Innovative Plastics, US LLC, was provided to an extrusion-based digital manufacturing system purchased from Stratysys, Inc and known as FORTUSTM-400 mc.

The consumable filament had a length, an exterior surface, and a plurality of tracks along at least a portion of the length, such that the plurality of tracks provided a fractal dimensionality for at least a portion of the exterior surface that is greater than two for a length scale between 0.01 millimeters and 1.0 millimeter. The teeth of a rotatable drive mechanism retained by the extrusion-based digital manufacturing system engaged with a rotatable drive mechanism with the plurality of tracks of the consumable filament. Portions of the consumable filament were fed successively with the rotatable drive mechanism to a liquefier retained by the extrusion-based digital manufacturing system. Successive teeth of the rotatable drive mechanism were continuously engaged with successive tracks of the plurality of tracks while feeding the successive portions of the consumable filament. The consumable filament melted in the liquefier to provide a melted consumable material. The melted consumable material from the liquefier was extruded and the extruded consumable material was deposited in a layer-by-layer manner to form the separator spline.

The additive manufacturing process described above was used to fabricate parts with an "X" cross-section with nominal dimensions of 4.7 mm tip-to-tip and fin thickness of nominally 1.0 mm. The fabricated parts had a nominal length of 127 mm. Different machine settings were used (changing contour and raster dimensions) to produce parts which varied in mass from 1.03 to 1.20 g.

This length was limited by the dimensional capabilities of the equipment used, and it should be appreciated that longer lengths could be fabricated with appropriately sized equipment.

Example 9 illustrates that separator spline parts can be fabricated using an additive manufacturing process. Our results show that additive manufacturing processes make articles having reduced density, as compared with separator splines that are solid and made from ULTEM 9085 and that have the same dimensions as those made from the additive manufacturing process. The expected weight of a solid part with the described dimensions fabricated with ULTEM 9085, for instance, is 1.43 g. As such, the separator splines made by additive manufacturing represented a density reduction ranging from 16% to 28%. No blowing agent was used in this process so the density reduction is due to the open lattice structure produced as material is placed by the additive manufacturing equipment.

The materials of the foregoing examples can meet or exceed regulatory requirements for data communications cable, e.g., the Underwriter's Laboratory Standard UL-910 Plenum Test, or NFPA 262. UL-910 Plenum Test is as follows. A plenum is defined as any space used as part of an air-handling system. This includes heating/air-conditioning ducts and air returns, which frequently include the space between suspended ceilings and the floor above in modern office buildings. The National Electric Code (NEC) requires that "exposed cables (those not in conduit) in plenums be listed as having adequate fire-resistant and low-smoke producing characteristics ..."

A "Standard For Test Method For Fire and Smoke Characteristics of Cables Used in Air-Handling Spaces" was developed by Underwriters' Laboratories (UL) to classify cables for this NEC requirement. This test is performed in a 25 foot Stein Tunnel test furnace (also specified in ASTM E-84 test for building materials). Designed to match the rigors of the application, this test is quite demanding.

In the UL-910 test, a single layer of 24 foot lengths of cable are supported by a one foot wide cable rack, which is filled with cables. The cables are ignited by an 88 K W (300,000 BTU/hr) methane flame. Flame spread is aided by a 240 ft/min draft. During the 20 minute test, flame spread is observed through small windows spaced one foot apart. Smoke is measured by a photocell installed in the exhaust duct.

To qualify, cables must have a flame spread of less than 5 feet beyond the end of the 4 1/2 foot ignition flame, a peak optical density of 0.5 maximum (33% light transmission) and a maximum average optical density of 0.15 (70% light transmission).

In summary, disclosed herein is an article comprising a foamed, polymeric, separator spline shaped to isolate at least one twisted pair of conductors, optionally wherein the foamed separator spline has a reduced density as compared to a non-foamed solid, separator spline; optionally, wherein the foamed polymeric separator spline is one selected from a foamed polyetherimide (PEI), a foamed polyetherimide/polysiloxane copolymer, a foamed thermoplastic-elastomer-modified-polyphenylene-ether blend, and combinations thereof optionally wherein the separator spline has a length ranging from 1 meter to 5000 meters and a cross sectional dimension ranging from 0.1 mm to 5 mm, and a thickness ranging from 0.1 to 5 mm; optionally wherein the shape of the separator spline is selected from one of the following shapes: (i) a +, (2) an X, (iii) a rod, (iv) a star configuration, (v) tube, (vi) flat rectangular, for example wherein one twisted pair of conductors is present in each of the arms of the + and the X; and optionally wherein the separator spline comprises a foamed polyetherimide (PEI) having a density reduction as compared to solid PEI ranging from about 3% to about 65% optionally wherein the separator spline comprises a foamed polyetherimide (PEI) having a density reduction as compared to solid PEI ranging from about 3% to about 55%.

Also disclosed is a cable comprising the separator spline of any one of the foregoing embodiments, and a plurality of the twisted conductor pairs encased in a sheath, optionally wherein the cable meets or exceeds at least one of UL-910 Plenum Test and NFPA 262; optionally wherein the cable is a data communication cable and the plurality of twisted conductor pairs is equal to four; optionally wherein the sheath also comprises one selected from the group consisting of a foamed polyetherimide (PEI), a foamed polyetherimide/polysiloxane copolymer, a foamed thermoplastic-elastomer-modified-polyphenylene-ether blend, and combinations thereof; and optionally wherein the foamed separator spline has a compressive strength ranging from 15 to less than 124 MPa, specifically a compressive strength of 27 to 84 MPa; optionally wherein the dielectric constant of the separator spline material is from about 2.0 to less than 3.15; optionally wherein the separator spline has a shape selected from +-shape, an X-shape, and a flat tape-shape, for example wherein one twisted pair of conductors is present in each of the arms of the + and the X.

In another embodiment, an article comprises a halogen-free separator spline for isolating at least two twisted pair of communication conductors to reduce cross-talk between the conductors, the article comprising: two twisted pairs of communication conductors, a foamed, halogen-free separator spline, the separator spline being interposed between the two pairs of communication conductors, the separator spline comprising a foamed polyetherimide (PEI) or a polyetherimide/siloxane copolymer, wherein the foam reduces the density, as compared to a corresponding non-foamed polymer, in the range of about 3% to about 55%; optionally further comprising a sheath covering the separator spline and the communication conductors.

Still further disclosed is a lightweight, flame and smoke retardant communication cable comprising at least two twisted pairs of communication conductors, separated by a halogen-free, foamed polymeric separator spline, the twisted pairs and spline being sheathed by an outer covering, optionally wherein the at least two twisted pairs range from two to sixteen twisted pairs; optionally wherein the separator spline has a shape selected from +-shape, an X-shape, and a flat tape-shape, for example wherein one twisted pair of conductors is present in each of the arms of the + and the X.

In another embodiment, a communication cable comprises a plurality of twisted conductor pairs, the conductor pairs being separated by a separator spline, wherein the separator spline has improved smoke, flame, and reduced toxicity properties; wherein the separator spline comprises a melt processed, foamed, polyetherimide (PEI) component selected from the group of polyetherimide homopolymers, polyetherimide copolymers, and combinations thereof, the separator spline having a reduced density, as compared to non-foamed PEI, of from about 3% to about 55%, optionally wherein the polyetherimide copolymercomprises a polyetherimide/polysiloxane copolymer; optionally wherein the dielectric constant of the separator spline material is from about 2.0 to less than 3.15; optionally wherein the separator spline has a shape selected from +-shape, an X-shape, and a flat tape-shape, for example wherein one twisted pair of conductors is present in each of the arms of the + and the X.

A method for making the article or cable of any one of the foregoing embodiments comprises extruding a composition through a shaped die, the composition comprising (i) a blowing agent, (ii) a thermoplastic polymer selected from the group of polyetherimide (PEI), polyetherimide/polysiloxane copolymer, elastomer-modified-polyphenylene-ether blend, and combinations thereof, and optionally a nucleating agent.

Another embodiment is the any of the foregoing articles wherein the separator spline is made in an extrusion-based digital manufacturing system, the method comprising: providing a consumable filament of the polymeric material to the extrusion-based digital manufacturing system, the consumable filament having a length, an exterior surface, and a plurality of tracks along at least a portion of the length, wherein the plurality of tracks provide a fractal dimensionality for at least a portion of the exterior surface that is greater than two for a length scale between 0.01 millimeters and 1.0 millimeter; engaging teeth of a rotatable drive mechanism retained by the extrusion-based digital manufacturing system with the plurality of tracks of the consumable filament; feeding successive portions of the consumable filament with the rotatable drive mechanism to a liquefier retained by the extrusion-based digital manufacturing system, wherein successive teeth of the rotatable drive mechanism are continuously engaged with successive tracks of the plurality of tracks while feeding the successive portions of the consumable filament; melting the consumable filament in the liquefier to provide a melted consumable material; extruding the melted consumable material from the liquefier; and depositing the extruded consumable material in a layer-by-layer manner to form at least a portion of the separator spline.

In still another embodiment, any of the foregoing articles can have the separator spline comprising an amorphous polymer composition comprising (a) a polyetherimide, and (b) a phosphorus-containing stabilizer, in an amount that is effective to increase the melt stability of the polyetherimide, wherein the phosphorus-containing stabilizer exhibits a low volatility such that, as measured by thermogravimetric analysis of an initial amount of a sample of the phosphorus-containing stabilizer, greater than or equal to 10 percent by weight of the initial amount of the sample remains unevaporated upon heating of the sample from room temperature to 300° C. at a heating rate of a 20° C. per minute under an inert atmosphere, optionally wherein the phosphorous-containing stabilizer has a formula P-R'ₐ, where R' is independently H, alkyl, alkoxy, aryl, aryloxy, or oxy substituent and a is 3 or 4.

Unless expressly specified herein, all percentages are percent by weight. All molecular weights are weight average molecular weight unless otherwise specified herein.

## Claims

1. An extruded separator spline of indeterminate length for separating at least two pairs of twisted conductors comprising an extrudate having an indeterminate length; said extrudate having a central longitudinal axis along its indeterminate length; and wherein the extrudate is formed of a foamed, polymeric, halogen-free material and further wherein the extrudate has
a. a shape having four arms emanating from the central longitudinal axis; the extrudate further comprising a cross-section without a continuous void along either the longitudinal axis or in any of said four arms; each of the arms being of uniform dimension from the longitudinal axis towards a terminal end of each arm; each of the arms being arranged in an angular disposition relative to the other arms of the extrudate and adjacent arms defining a space therebetween such that a twisted pair of conductors can nest in the space without extending beyond the terminal ends of the adjacent arms; or
b. a shape being selected from the group consisting of a rod, a star, and a bar; a periphery of each of the rod, the star and the bar having a plurality of cavities extending from the periphery into the body of the rod, the star and the bar; said cavities being of a size and shape to house within the cavity a twisted pair of conductors; the extrudate further comprising a cross-section without a continuous void along the longitudinal axis, and wherein the extrudate forms a separator spline suitable to isolate at least two twisted pair of conductors in a different cavity of said plurality of cavities.

2. The article according to claim 1, wherein the foamed polymeric separator spline is one selected from a foamed polyetherimide (PEI), a foamed polyetherimide/polysiloxane copolymer, a foamed thermoplastic-elastomer-modified-polyphenylene-ether blend, and combinations thereof.

3. The article of any one of claims 1 to 2, wherein the separator spline has a length ranging from 1 meter to 5000 meters and a cross sectional dimension ranging from 0.1 mm to 5 mm, and a thickness ranging from 0.1 to 5 mm.

4. The article of any one of claims 1 to 3, wherein the separator spline comprises a foamed polyetherimide (PEI) having a density reduction as compared to solid PEI ranging from about 3% to about 65%.

5. A cable comprising the separator spline of any one of claims 1 to 4 and a plurality of the twisted conductor pairs encased in a sheath.

6. The cable of Claim 5, wherein the cable meets or exceeds at least one ofUL-910 Plenum Test and NFPA 262.

7. The cable of any one of claims 5 to 6, wherein the cable is a data communication cable and the plurality of twisted conductor pairs is equal to four.

8. The cable of any one of claims 5 to 7, wherein the sheath also comprises one selected from the group consisting of a foamed polyetherimide (PEI), a foamed polyetherimide/polysiloxane copolymer, a foamed thermoplastic-elastomer-modified-polyphenylene-ether blend, and combinations thereof.

9. The communication cable of any one of claims 5 to 8, wherein the foamed separator spline has a compressive strength ranging from 15 to less than 124 MPa.

10. The communication cable of any one of claims 5 to 8, wherein the foamed separator spline has a compressive strength of 27 to 84 MPa.

11. A method for making the article of any one of claims 1 to 10, comprising extruding a composition through a shaped die, the composition comprising (i) a blowing agent, (ii) a thermoplastic polymer selected from the group of polyetherimide (PEI), polyetherimide/polysiloxane copolymer, elastomer-modified-polyphenylene-ether blend, and combinations thereof, and optionally a nucleating agent.

12. The article of any one of claims 1 to 10, wherein the separator spline is made in an extrusion-based digital manufacturing system, the method comprising:
providing a consumable filament of the polymeric material to the extrusion-based digital manufacturing system, the consumable filament having a length, an exterior surface, and a plurality of tracks along at least a portion of the length, wherein the plurality of tracks provide a fractal dimensionality for at least a portion of the exterior surface that is greater than two for a length scale between 0.01 millimeters and 1.0 millimeter;
engaging teeth of a rotatable drive mechanism retained by the extrusion-based digital manufacturing system with the plurality of tracks of the consumable filament;
feeding successive portions of the consumable filament with the rotatable drive mechanism to a liquefier retained by the extrusion-based digital manufacturing system, wherein successive teeth of the rotatable drive mechanism are continuously engaged with successive tracks of the plurality of tracks while feeding the successive portions of the consumable filament;
melting the consumable filament in the liquefier to provide a melted consumable material;
extruding the melted consumable material from the liquefier; and
depositing the extruded consumable material in a layer-by-layer manner to form at least a portion of the separator spline.

13. The article of any one of claims 1 to 10, wherein the separator spline comprises an amorphous polymer composition comprising (a) a polyetherimide, and (b) a phosphorus-containing stabilizer, in an amount that is effective to increase the melt stability of the polyetherimide, wherein the phosphorus-containing stabilizer exhibits a low volatility such that, as measured by thermogravimetric analysis of an initial amount of a sample of the phosphorus-containing stabilizer, greater than or equal to 10 percent by weight of the initial amount of the sample remains unevaporated upon heating of the sample from room temperature to 300° C. at a heating rate of a 20° C. per minute under an inert atmosphere.

14. The article of Claim 13, wherein the phosphorous-containing stabilizer has a formula P-R'ₐ, where R' is independently H, alkyl, alkoxy, aryl, aryloxy, or oxy substituent and a is 3 or 4.

## Patentansprüche

1. Extrudiertes Trennkeilelement unbestimmter Länge zum Trennen von mindestens zwei Paaren verdrillter Leiter, umfassend ein Extrudat mit unbestimmter Länge; wobei das Extrudat eine mittige Längsachse entlang seiner unbestimmten Länge aufweist; und wobei das Extrudat aus einem geschäumten, polymeren, halogenfreien Material ausgebildet ist und wobei das Extrudat ferner Folgendes aufweist:
a. eine Form mit vier aus der mittigen Längsachse austretenden Armen; wobei das Extrudat ferner einen Querschnitt ohne einen durchgehenden Leerraum entweder entlang der Längsachse oder in irgendeinem der vier Arme umfasst; wobei jeder der Arme eine gleichmäßige Abmessung von der Längsachse zu einem fernen Ende jedes Arms aufweist; wobei jeder der Arme in einer Winkelanordnung relativ zu den anderen Armen des Extrudats angeordnet ist und benachbarte Arme einen Raum zwischen sich derart definieren, dass ein verdrilltes Leiterpaar in dem Raum aufgenommen sein kann, ohne sich über die fernen Enden der benachbarten Arme hinaus zu erstrecken; oder
b. eine Form, die aus der Gruppe bestehend aus einer Stange, einem Stern und einem Stab ausgewählt ist; wobei ein Rand von jeweils der Stange, dem Stern und dem Stab eine Vielzahl von Vertiefungen aufweist, die sich vom Rand in den Körper der Stange, des Sterns und des Stabs erstrecken; wobei Vertiefungen eine Größe und Form derart aufweisen, dass sie ein verdrilltes Leiterpaar in der Vertiefung aufnehmen; wobei das Extrudat ferner einen Querschnitt ohne einen durchgehenden Leerraum entlang der Längsachse umfasst und wobei das Extrudat ein Trennkeilelement bildet, das zum Isolieren von mindestens zwei verdrillten Leiterpaaren in einer unterschiedlichen Vertiefung der Vielzahl von Vertiefungen geeignet ist.

2. Artikel nach Anspruch 1, wobei das geschäumte, polymere Trennkeilelement eines ist, das aus einem geschäumten Polyetherimid (PEI), einem geschäumten Polyetherimid-Polysiloxan-Copolymer, einer geschäumten Mischung aus einem mit thermoplastischem Elastomer modifiziertem Polyphenylenether und Kombinationen davon ausgewählt ist.

3. Artikel nach irgendeinem der Ansprüche 1 bis 2, wobei das Trennkeilelement eine von 1 Meter bis 5000 Meter reichende Länge, eine von 0,1 mm bis 5 mm reichende Querschnittsabmessung und eine von 0,1 bis 5 mm reichende Dicke aufweist.

4. Artikel nach irgendeinem der Ansprüche 1 bis 3, wobei das Trennkeilelement ein geschäumtes Polyetherimid (PEI) mit einer Dichteverringerung im Vergleich zu einem festen PEI aufweist, die von ungefähr 3 % bis ungefähr 65 % reicht.

5. Kabel umfassend das Trennkeilelement nach irgendeinem der Ansprüche 1 bis 4 und eine Vielzahl der verdrillten Leiterpaare, die in einer Ummantelung umschlossen sind.

6. Kabel nach Anspruch 5, wobei das Kabel mindestens eines von dem Plenum-Test UL-910 und NFPA 262 erfüllt oder übertrifft.

7. Kabel nach irgendeinem der Ansprüche 5 bis 6, wobei das Kabel ein Datenkommunikationskabel ist und die Vielzahl verdrillter Leiterpaare gleich vier ist.

8. Kabel nach irgendeinem der Ansprüche 5 bis 7, wobei die Ummantelung auch eines umfasst, das aus der Gruppe bestehend aus einem geschäumten Polyetherimid (PEI), einem geschäumten Polyetherimid-Polysiloxan-Copolymer, einer geschäumten Mischung aus einem mit thermoplastischem Elastomer modifiziertem Polyphenylenether und Kombinationen davon ausgewählt ist.

9. Kommunikationskabel nach irgendeinem der Ansprüche 5 bis 8, wobei das geschäumte Trennkeilelement eine von 15 bis weniger als 124 MPa reichende Druckfestigkeit aufweist.

10. Kommunikationskabel nach irgendeinem der Ansprüche 5 bis 8, wobei das geschäumte Trennkeilelement eine Druckfestigkeit von 27 bis 84 MPa aufweist.

11. Verfahren zur Herstellung des Artikels nach irgendeinem der Ansprüche 1 bis 10, umfassend das Extrudieren einer Zusammensetzung durch eine Formdüse, wobei die Zusammensetzung Folgendes umfasst: (i) ein Treibmittel, (ii) ein thermoplastisches Polymer, das aus der Gruppe von Polyetherimid (PEI), Polyetherimid-Polysiloxan-Copolymer, einer Mischung aus einem mit einem Elastomer modifiziertem Polyphenylenether und Kombinationen davon ausgewählt ist, und gegebenenfalls einen Keimbildner.

12. Artikel nach irgendeinem der Ansprüche 1 bis 10, wobei das Trennkeilelement in einem extrusionsbasierten digitalen Fertigungssystem hergestellt ist, wobei das Verfahren Folgendes umfasst:
Bereitstellen eines verbrauchbaren Filaments des polymeren Materials zu dem extrusionsbasierten digitalen Fertigungssystem, wobei das verbrauchbare Filament eine Länge, eine Außenfläche und eine Vielzahl von Profilen entlang zumindest einem Abschnitt der Länge aufweist, wobei die Vielzahl von Profilen eine fraktale Dimensionalität für zumindest einen Abschnitt der Außenfläche bereitstellt, die größer als zwei für eine Längenskala zwischen 0,01 Millimetern und 1,0 Millimeter ist;
Ineingriffbringen von Zähnen eines von dem extrusionsbasierten digitalen Fertigungssystem gehaltenen drehbaren Antriebsmechanismus mit der Vielzahl von Profilen des verbrauchbaren Filaments;
Zuführen aufeinanderfolgender Abschnitte des verbrauchbaren Filaments mit dem drehbaren Antriebsmechanismus zu einem von dem extrusionsbasierten digitalen Fertigungssystem gehaltenen Verflüssiger, wobei aufeinanderfolgende Zähne des drehbaren Antriebsmechanismus kontinuierlich mit aufeinanderfolgenden Profilen der Vielzahl von Profilen in Eingriff gebracht werden, während die aufeinanderfolgenden Abschnitte des verbrauchbaren Filaments zugeführt werden;
Schmelzen des verbrauchbaren Filaments in dem Verflüssiger, um ein geschmolzenes verbrauchbares Material bereitzustellen;
Extrudieren des geschmolzenen verbrauchbaren Materials aus dem Verflüssiger; und
schichtweises Austragen des extrudierten verbrauchbaren Materials, um zumindest einen Abschnitt des Trennkeilelements zu bilden.

13. Artikel nach irgendeinem der Ansprüche 1 bis 10, wobei das Trennkeilelement eine amorphe Polymerzusammensetzung umfasst, die (a) ein Polyetherimid und (b) einen phosphorhaltigen Stabilisator in einer Menge umfasst, die die Schmelzstabilität des Polyetherimids wirksam erhöht, wobei der phosphorhaltige Stabilisator ein niedrige Flüchtigkeit derart zeigt, dass bei Messung durch thermogravimetrische Analyse einer Anfangsmenge einer Probe des phosphorhaltigen Stabilisators mehr als oder gleich 10 Gewichtsprozent der Anfangsmenge der Probe bei Erhitzung der Probe von Raumtemperatur auf 300 °C bei einer Aufheizgeschwindigkeit von 20 °C pro Minute unter einer inerten Atmosphäre unverdampft bleiben.

14. Artikel nach Anspruch 13, wobei der phosphorhaltige Stabilisator eine Formel P-R'ₐ aufweist, wobei R' unabhängig für einen H-, Alkyl-, Alkoxy-, Aryl-, Aryloxy- oder Oxy-Substituenten steht und a für 3 oder 4 steht.

## Revendications

1. Languette séparatrice expansée de longueur indéterminée pour séparer au moins deux paires de conducteurs torsadés comprenant un extrudat ayant une longueur indéterminée ; ledit extrudat ayant un axe longitudinal central le long de sa longueur indéterminée ; et dans laquelle l'extrudat est formé d'un matériau polymère, exempt d'halogènes, expansé, et en outre dans laquelle l'extrudat présente
a. une forme ayant quatre bras émanant de l'axe longitudinal central ; l'extrudat comprenant en outre une section transversale dépourvue de vide continu le long de l'axe longitudinal ou dans l'un quelconque desdits quatre bras ; chacun des bras ayant une dimension uniforme depuis l'axe longitudinal vers une extrémité terminale de chaque bras ; chacun des bras étant agencé selon une disposition angulaire par rapport aux autres bras de l'extrudat et aux bras adjacents définissant un espace entre eux de sorte qu'une paire torsadée de conducteurs puisse s'emboîter dans l'espace sans s'étendre au-delà des extrémités terminales des bras adjacents ; ou
b. une forme étant choisie dans le groupe constitué par une tige, une étoile et une barre ; une périphérie de chacune de la tige, l'étoile et la barre présentant une pluralité de cavités s'étendant depuis la périphérie dans le corps de la tige, de l'étoile et de la barre ; lesdites cavités ayant une taille et une forme permettant de loger dans la cavité une paire torsadée de conducteurs ; l'extrudat comprenant en outre une section transversale dépourvue de vide continu le long de l'axe longitudinal, et dans lequel l'extrudat forme une languette séparatrice apte à isoler au moins deux paires de conducteurs torsadées dans une cavité différente de ladite pluralité de cavités.

2. Article selon la revendication 1, dans lequel la languette séparatrice polymère expansée est une languette choisie parmi un polyétherimide (PEI) expansé, un copolymère de polyétherimide/polysiloxane expansé, un mélange de polyphénylène-éther modifié par un élastomère thermoplastique expansé, et leurs combinaisons.

3. Article selon l'une quelconque des revendications 1 à 2, dans lequel la languette séparatrice a une longueur allant de 1 mètre à 5 000 mètres et une dimension en coupe transversale allant de 0,1 mm à 5 mm, et une épaisseur allant de 0,1 à 5 mm.

4. Article selon l'une quelconque des revendications 1 à 3, dans lequel la languette séparatrice comprend un polyétherimide (PEI) expansé ayant une réduction de densité par rapport à un PEI solide allant d'environ 3 % à environ 65 %.

5. Câble comprenant la languette séparatrice selon l'une quelconque des revendications 1 à 4 et une pluralité de paires de conducteurs torsadées enfermées dans une gaine.

6. Câble selon la revendication 5, dans lequel le câble satisfait ou dépasse au moins l'un des tests UL-910 Plenum Test et NFPA 262.

7. Câble selon l'une quelconque des revendications 5 à 6, dans lequel le câble est un câble de communication de données et la pluralité de paires de conducteurs torsadées est égale à quatre.

8. Câble selon l'une quelconque des revendications 5 à 7, dans lequel la gaine comprend également un constituant choisi dans le groupe constitué par un polyétherimide (PEI) expansé, un copolymère de polyétherimide/polysiloxane expansé, un mélange de polyphénylène-éther modifié par un élastomère thermoplastique expansé, et leurs combinaisons.

9. Câble de communication selon l'une quelconque des revendications 5 à 8, dans lequel la languette séparatrice expansée présente une résistance à la compression allant de 15 à moins de 124 MPa.

10. Câble de communication selon l'une quelconque des revendications 5 à 8, dans lequel la languette séparatrice expansée présente une résistance à la compression de 27 à 84 MPa.

11. Procédé de fabrication de l'article selon l'une quelconque des revendications 1 à 10, comprenant l'extrusion d'une composition à travers une filière façonnée, la composition comprenant (i) un agent d'expansion, (ii) un polymère thermoplastique choisi dans le groupe constitué par un polyétherimide (PEI), un copolymère de polyétherimide/polysiloxane, un mélange de polyphénylène-éther modifié par un élastomère, et leurs combinaisons, et éventuellement un agent de nucléation.

12. Article selon l'une quelconque des revendications 1 à 10, dans lequel la languette séparatrice est fabriquée dans un système de fabrication numérique fondé sur l'extrusion, le procédé comprenant :
la fourniture d'un filament consommable du matériau polymère au système de fabrication numérique fondé sur l'extrusion, le filament consommable ayant une longueur, une surface extérieure et une pluralité de pistes le long d'au moins une partie de la longueur, dans laquelle la pluralité de pistes fournissent une dimensionnalité fractale pour au moins une partie de la surface extérieure qui est supérieure à deux pour une échelle de longueur comprise entre 0,01 millimètre et 1,0 millimètre ;
la mise en prise des dents d'un mécanisme d'entraînement rotatif retenu par le système de fabrication numérique fondé sur l'extrusion avec la pluralité de pistes du filament consommable ;
l'alimentation de portions successives du filament consommable avec le mécanisme d'entraînement rotatif dans un liquéfacteur retenu par le système de fabrication numérique fondé sur l'extrusion, dans laquelle les dents successives du mécanisme d'entraînement rotatif sont en prise continue avec des pistes successives de la pluralité de pistes tout en alimentant les parties successives du filament consommable ;
la fusion du filament consommable dans le liquéfacteur pour obtenir un matériau consommable fondu ;
l'extrusion du matériau consommable fondu à partir du liquéfacteur ; et
le dépôt du matériau consommable extrudé couche par couche pour former au moins une partie de la languette séparatrice.

13. Article selon l'une quelconque des revendications 1 à 10, dans lequel la languette séparatrice comprend une composition de polymère amorphe comprenant (a) un polyétherimide, et (b) un stabilisant contenant du phosphore, en une quantité qui est efficace pour augmenter la stabilité à l'état fondu du polyétherimide, dans lequel le stabilisant contenant du phosphore présente une volatilité faible telle que mesurée par analyse thermogravimétrique d'une quantité initiale d'un échantillon du stabilisant contenant du phosphore, une quantité supérieure ou égale à 10 % en poids de la quantité initiale de l'échantillon reste non évaporée lors du chauffage de l'échantillon de la température ambiante à 300 °C à une vitesse de chauffage de 20 °C par minute sous une atmosphère inerte.

14. Article selon la revendication 13, dans lequel le stabilisant contenant du phosphore répond à la formule P-R'ₐ, où R' est indépendamment un substituant H, alkyle, alcoxy, aryle, aryloxy ou oxy et a est 3 ou 4.
